

Patented Dec. 28, 1926.

1,612,671

## UNITED STATES PATENT OFFICE.

FERNANDO SOMOZA VIVAS, OF LOS ANGELES, CALIFORNIA.

## FIREPROOF PAINT.

No Drawing. Application filed June 14, 1923, Serial No. 645,341. Renewed May 26, 1926.

The invention relates to paints and has as an object the provision of a fire proof paint which shall be absolutely non-inflammable.

5 A further object of the invention is the provision of a paint which will not only protect the material to which it is applied from fire but will also be effective to perform the usual function of paint by protecting the 10 material to which it is applied from the effects of weather or wear.

A further object of the invention is the provision of paint which is applicable not only to wood but to paper and all other inflammable materials. A further object of the invention is the provision of a paint which will have a high gloss which is not affected by the action of the elements. The formula which is preferred as a physical 15 embodiment of the invention comprises the following ingredients in the proportions named:—

|                     | Parts. |
|---------------------|--------|
| Drying oil          | 75     |
| 25 Zinc white       | 40     |
| Lead sulphate       | 20     |
| Lead carbonate      | 20     |
| Silica or kaolin    | 10     |
| Borax               | 10     |
| 30 Potash alum      | 10     |
| Boric acid          | 5      |
| Tungstate of sodium | 5      |
| Thinner (No. 3)     | 5      |

35 The thinner listed in the above formula is made the subject matter of a separate application, Serial No. 645,346 filed June 14, 1923, the formula of which is as follows:

|                         | Parts |
|-------------------------|-------|
| 40 "Nearturps"          | 40    |
| Turpentine              | 10    |
| Zinc sulphate           | 5     |
| Hexachlorethane         | 1     |
| Drying oil              | 4     |
| 45 Carbon tetrachloride | 40    |

In the formula for the paint above given zinc white is listed which it is preferred to use as being resistant to fumes particularly 50 of ammonia. It will be understood that

white lead may be substituted for this material if so desired.

By the term "Nearturps" used in the above formula, a hydrocarbon is referred to which is a gasoline produced by a straight distillation process and which has been deodorized by treatment with alcohol.

The silica or kaolin in the above formula is utilized as an inert filler and may be replaced by many other materials in finely divided condition which are sufficiently inexpensive and which are inert. Because of their cheapness many forms of earthy material may be desirably used. While a small proportion of thinner is recited, it will be understood that if the paint has the desired consistency without the thinner the same may be omitted without detriment to the fireproof qualities of the paint.

Minor changes may be made in the proportions of parts and known equivalents may be substituted for some of the ingredients named without departing from the spirit of the invention.

I claim:

1. A fireproof paint comprising in combination, drying oil, zinc white, lead sulphate, lead carbonate, finely divided inert filling material, borax, potash alum, boric acid, tungstate of sodium and a thinner in 80 proportions to produce a fire-proof paint.

2. A fireproof paint comprising in combination, drying oil, 75 parts, zinc white, 40 parts, lead sulphate, 20 parts, lead carbonate, 20 parts, inert filling material, 10 parts, borax, 10 parts, potash alum, 10 parts, boric acid, 5 parts and tungstate of sodium, 5 parts.

3. A fireproof paint comprising in combination, drying oil, 75 parts, zinc white, 40 parts, lead sulphate, 20 parts, lead carbonate, 20 parts, inert filling material, 10 parts, borax, 10 parts, potash alum, 10 parts, boric acid, 5 parts, tungstate of sodium, 5 parts, and 5 parts of a thinner comprising "Nearturps," 40 parts, turpentine, 10 parts, zinc sulphate, 5 parts, hexachlorethane, 1 part, drying oil, 4 parts and carbon tetrachloride, 40 parts.

FERNANDO SOMOZA VIVAS.

75

90

95

5054  
X320